

Oct. 24, 1967

J. M. GESS

3,348,970

ELECTROSTATIC CONDUCTIVE PAPER

Filed Jan. 16, 1962



INVENTOR.  
JEROME M. GESS  
BY  
*Harold Jenkins*  
ATTORNEY

# United States Patent Office

3,348,970

Patented Oct. 24, 1967

1

3,348,970

ELECTROSTATIC CONDUCTIVE PAPER  
Jerome M. Gess, Drexel Hill, Pa., assignor to Scott Paper  
Company, Philadelphia, Pa., a corporation of Pennsyl-  
vania

Filed Jan. 16, 1962, Ser. No. 166,497  
5 Claims. (Cl. 117—201)

The present invention relates to a novel recording medium and more particularly to an electrically conducting paper useful in the electrostatic printing art.

The basic principles of electrostatic printing are quite simple. An electrostatic charge is imparted to paper or other dielectric material in a predetermined pattern which is subsequently made visible by dusting with a powder carrying an opposite charge. The powder is attracted to the charged areas of the paper to make the latent charge image visible. The powder can be permanently fused to the paper by heat, pressure or other means.

Where in the electrostatic printing the electrically recording paper is subjected to a modulated voltage to create the latent image in accordance with the intensity of the voltage, the recording paper includes a base sheet coated upon opposite sides with dielectrical and conductive layers with a sealing media interposed therebetween to prevent migration of the conductive material into the dielectric. Manifestly, the inclusion of additional lamina in a composite sheet adds to the cost of production thereof and also creates a source of potential product deterioration.

However, the preparation of an electrostatic image recording paper in which the dielectric layer is directly superposed upon the conductive paper base has necessitated the development of a specialized combination of chemical additives which will impart to the paper good electroconductivity over a relatively wide range of relative humidities, which will readily be incorporated in said base paper and which will be resistant to migration therefrom.

It is, therefore, a primary object of my invention to provide an electrostatic image recording medium composed of a dielectric coating applied directly to an electrically conducting paper sheet.

Another object of my invention is to provide an electrically conductive paper having a specific conductivity of from  $10^7$  to  $10^{10}$  ohms in which the sensitizing agent of the paper exhibits exceptional stability against migrating forces.

A still further object of the present invention is to provide an improved electrostatic image recording medium, composed of an electrically conducting paper surfaced with a dielectric, the composite having a specific electrical conductivity in the range of from  $10^{11}$  to  $10^{14}$  ohms.

Other objects and advantages of my invention will be readily apparent from the following detailed description of certain preferred embodiments thereof when taken in conjunction with the accompanying drawing wherein the single figure represents a fragmentary perspective view of a recording sheet as contemplated by the invention.

I have discovered that the water soluble quaternary ammonium compounds when supplemented by the admixture therewith of relatively lesser amounts of one or more deliquescent salts, such as for example lithium chloride will impart electric conductivity to paper and will function adequately over a wide range of relative humidities in the transfer of an electrostatic charge to a dielectric coating thereon and the formation of latent image patterns.

The quaternary ammonium compounds suitable for incorporation in the paper base of the present invention are those which have the general formula:

2



5 wherein  $R_1$ ,  $R_2$  and  $R_3$  are low molecular alkyl groups, particularly methyl and ethyl groups,  $R_4$  is a long chain aliphatic hydrocarbon or mixed aliphatic and aromatic nucleus containing from 8 to 21 carbon atoms, and  $X$  is a halogen or nitrate group.

10 Among the quaternary ammonium compounds which are represented in their essential by the foregoing formulas are the following:

Alkyl polyethoxyethanol benzyl ammonium chloride available as Katapone VV 328.

15 N-alkyl ( $C_{10-18}$ ) oxyhydroxy propyl trimethyl ammonium chloride.

Lauryl oxyhydroxy propyl trimethyl ammonium chloride. Alkyl dimethyl 3,4 dichloro benzyl ammonium chloride, Tetrosan 3,4D.

20 Stearamido propyl dimethyl, beta hydroxy ethyl ammonium nitrate sold under the tradename Catanac SN. Cetyl-oxyhydroxy propyl trimethyl ammonium chloride. N-alkyl dimethyl methylbenzyl ammonium chloride, sold under the tradename BTc-471.

25 The deliquescent salts suitable for admixture with the quaternary amines and incorporation in the base stratum of an electroconducting paper include lithium chloride, lithium bromide, calcium chloride, and magnesium chloride. The presence of these salts in the impregnating solution permits a reduction in the amount of quaternary amine necessary to impart the desired level of conductivity to the paper base and accordingly enables a material reduction in the cost of manufacture of the ultimate image recording medium.

30 A paper sheet 1, approximately  $2\frac{1}{2}$  mils caliper contains a mixture of a quaternary ammonium salt and a deliquescent salt in sufficient quantity to impart the desired specific electric conductivity to the paper sheet and carries on one side a film 2 of a dielectric material such as for example an alkali soluble polyvinylacetate resin.

35 The sequence of steps entailed in fabrication of the composite recording sheet is not critical. For example, the layer of dielectric material may be applied to one side of a web of paper from a coating bath or by air knife, coating or doctor blading and thereafter the opposite side of the coated sheet may be impregnated by spraying with a concentrated aqueous solution of the quaternary ammonium salt-deliquescent salt mixture. Alternatively, the base sheet may be impregnated with the salt solution prior to the application thereto of the dielectric coating material.

40 My invention is illustrated more specifically in the following examples which, however, are not to be construed as imposing any particular limitation thereon.

## Example I

An aqueous suspension composed of 60%, by weight, of alkali soluble polyvinyl acetate, 35%, by weight, of clay and 5%, by weight, of titanium dioxide in 400 cc. of 45 water containing 15 cc. of  $NH_4OH$  was applied as a coating to one side of a sheet of 48 pound/3000 square feet surface area bleached southern kraft paper by an air knife coater. The coating equipment was adjusted so that the paper sheet was advanced at a rate of approximately 25 feet per minute with the application of coating mixture controlled to approximately 12.8 pounds per 3000 square feet of surface area. After emergence from the coater, the sheet was dried at a temperature of from 300 to 350° F., cooled and reeled.

50 To complete the composite paper a solution containing 12%, by weight, of cetyl oxyhydroxy propyl trimethyl ammonium chloride and 3%, by weight, of lithium chloride

in isopropyl-alcohol was sprayed over the uncoated side of the dielectric surfaced paper previously prepared, using a Paasche automatic spray gun delivering 1.05 pounds of solution per ream of paper with the sheet traveling at 10 feet per minute through the spray. The sprayed sheet was passed between a pressure nip formed by opposed rolls of 40 durometer rubber of the Shore scale under 80 pounds per square inch pressure after which the sheet was again dried. The final composite sheet had a surface conductivity of  $10^8$  ohms.

The value of the finished sheet as an electrostatic image recording medium was evinced by the following test. A piece of letterpress type was superposed on the dielectric (resin coated) side of the sheet. The other side of the sheet contacted a metal platen. Upon connecting the piece of type to the negative pole of a constant voltage source and the metal platen to the positive pole thereof and passing a current of 1000 volts through the sheet there was created a latent electrostatic image in the paper. A developing powder dusted over the sheet was attracted to the charged portion of the paper to produce thereon a patterned image of the letterpress type and upon heating the developing powder was fused to form a permanent image.

*Example II*

A coating formulation prepared as in Example I was applied to 35 pounds/3000 square feet surface area paper by means of an air knife coater. The coater was run at 300 f.p.m. and 12.8 pounds dry weight of coating was applied per 3000 square feet surface area. The coating was dried by passing through a hot air oven at 300° F. and reeled. Subsequently a solution containing 10 parts, by weight, of stearyl oxyhydroxy propyl trimethyl ammonium chloride and 3 parts, by weight, of calcium chloride in isopropyl alcohol was applied by spraying to the uncoated side of this paper in an amount such that there was retained in the paper at least 1.35 pounds of the salt mixture per 3000 square feet of paper. The final paper recorded satisfactorily electrostatically induced images under 1000 volts and 50% relative humidity.

*Example III*

A bleached kraft having a basis weight of 35 pounds per 3000 square foot ream was impregnated with an aqueous solution containing 35%, by weight, of N-alkyl dimethyl methyl benzyl ammonium chloride and 10%, by weight, of lithium chloride so that there was retained in the sheet in excess of 3.5 pounds of the mixed salts per 3000 square feet. The impregnated paper was passed between a roll nip, dried at 300° F. and reeled.

This impregnated paper was subsequently coated with the coating formulation of Example I, and the coated paper containing about 12 pounds (dry weight) of the dielectric material per 3000 square feet of surface area was dried at 300° F. This final paper, which was considerably more opaque than the paper of Example II, also recorded satisfactorily electrostatically induced images.

It has been determined that the concentrations of mixed amine-deliquescent salt impregnates are not critical to the success of the present invention. For example, amounts in the range of from 0.5 to 10 pounds per 3000 square feet of paper have been employed in source concentrations of from 25 to 85%, by weight, and will vary within these limits depending upon the specific salts employed and the specific conductivity which is desired in the final product. Nor is the ratio between the quaternary amine and deliquescent salt in the salt mixture critical for successful results have been obtained with ratios varying from 2:1 to as high as 5:1. While the specific conductivity is of minor significance, it is preferred, however, that the basic

sheet exhibits an approximate specific conductivity between  $10^7$  and  $10^9$  ohms and the composite to have a specific conductivity of from  $10^{12}$  and  $10^{14}$  ohms measured by placing one electrode on the dielectric side and the second electrode on the conductive side of the sheet.

Papers varying in caliper within the range of 2 to 5 mils have been successfully employed in the formation of image recording sheets while the preferred range of caliper is from 2.5 to 3 mils. Although a bleach kraft composite of 65% pine and 35% gum will possess greater inherent strength because of the larger proportions of long fibers therein, my invention is not limited to such paper and other types and weights of sheeting are equally serviceable. As to the material forming the dielectric coating of the sheet, the alkali soluble polyvinylacetates constitute a well recognized class of synthetic resin suitable for such application. I do not wish to be limited to the particular resin, however, for other resins, such as ethyl cellulose, will serve equally as well. The dielectric coating may vary between 3.5 and 15 pounds per 3000 square feet of paper surface, and it is preferred to apply the dielectric in the case of the polyvinylacetate type in the range of from 5 to 8 pounds per 3000 square feet. Generally, as the percentage of dielectric surfacing is decreased, the capacity of the composite sheet to accept and retain a given electrostatic charge is impaired. Heavier coatings of dielectric are possible although these will merely increase production costs without the realization of corresponding improvement in reproduction characteristics.

30. What I claim is:

1. An electrostatic image-recording medium consisting of a cellulose web having dispersed therein an N-alkyl oxyhydroxy propyl trimethyl ammonium chloride wherein the alkyl group contains from 10 to 18 carbon atoms, said cellulose web containing a dispersed deliquescent salt, and carrying on one surface a layer of a dielectric material.
2. An electrostatic image-recording medium consisting of a cellulose web having dispersed therein stearamido propyl dimethyl, beta hydroxy ethyl ammonium nitrate, said cellulose web containing a dispersed deliquescent salt, and carrying on one surface a layer of a dielectric material.
3. An electrostatic image-recording medium consisting of a cellulose web having dispersed therein cetyl-oxyhydroxy propyl trimethyl ammonium chloride, said cellulose web containing a dispersed deliquescent salt, and carrying on one surface a layer of a dielectric material.
4. An electrostatic image-recording medium consisting of a cellulose web having dispersed therein lauryl oxyhydroxy propyl trimethyl ammonium chloride, said cellulose web containing a dispersed deliquescent salt, and carrying on one surface a layer of a dielectric material.
5. An electrostatic image-recording medium consisting of a cellulose web having dispersed therein stearyl oxyhydroxy propyl trimethyl ammonium chloride, said cellulose web containing a dispersed deliquescent salt, and carrying on one surface a layer of a dielectric material.

60. **References Cited**

UNITED STATES PATENTS

- |           |         |                                 |
|-----------|---------|---------------------------------|
| 2,626,877 | 8/1951  | Carnes.                         |
| 3,011,918 | 12/1961 | Silvernail et al. ----- 117—201 |
| 3,075,859 | 1/1963  | Relph et al. ----- 117—155      |
| 3,110,621 | 11/1963 | Doggett et al.                  |

ALFRED L. LEAVITT, Primary Examiner.

RICHARD D. NEVIUS, Examiner.

70. W. L. JARVIS, A. GOLIAN, Assistant Examiners.